

## UNITED STATES PATENT OFFICE

2,153,135

## YARN TREATING PROCESSES AND COMPOSITIONS THEREFOR

Joseph B. Dickey and James G. McNally, Rochester, N. Y., assignors to Eastman Kodak Company, Rochester, N. Y., a corporation of New Jersey

No Drawing. Application November 26, 1937,  
Serial No. 176,683

22 Claims. (Cl. 28—1)

This invention relates to the conditioning of textile yarns and more particularly to the conditioning of filaments and yarns composed of organic derivatives of cellulose such as cellulose acetate, cellulose acetate propionate, cellulose acetate butyrate, etc., to render them more amenable to textile operations such as knitting and the like.

As is well-known in the manufacture of yarns, particularly those composed of or containing cellulose organic derivatives, it is necessary to treat the yarn in order to reduce the tendency toward breakage of the individual filaments or fibers when they are subjected to various mechanical strains and to lubricate the yarn in order to facilitate handling in such operations as spinning, twisting, winding and reeling. In addition it is necessary to treat yarn to adapt it for use as warp or filling or for the manufacture of various types of knitted fabrics. In knitting, it is particularly important that the yarn be soft and pliable in order that it may conform readily to the contour of the needles and thus produce a closely knit fabric free from such defects as "stitch distortion", "pin holes", "laddering", and the like.

Heretofore it has been proposed to employ softening agents such as polyhydric alcohols and similar agents as ingredients of yarn conditioning or lubricating formulae, generally in connection with mineral, animal or vegetable oils. It has been found, however, that most of the known softening agents and the various formulae containing them have certain drawbacks, one of the most serious of which is high vapor pressure, and in some cases too drastic a solvent action on the yarn. Many of such agents possess slight or insufficient solvent power for the lubricants with which they are used and it is accordingly necessary to employ blending agents or emulsifying agents in order to obtain operable yarn treating formulae. In addition, many of the known softening and lubricating agents are insufficiently soluble in water to permit satisfactory removal by aqueous scour baths.

This invention has as its principal object to provide an entirely new class of yarn conditioning agents which are particularly adapted for the treatment of yarns composed of or containing organic derivatives of cellulose and capable of lubricating, softening and rendering such yarns more amenable to knitting and other textile operations. A further and specific object is to provide a class of conditioning agents which augment or assist the lubricating action of vari-

ous lubricants when applied to such yarns. A still further object is to provide yarn softening and lubricating formulas which can be readily removed from the yarns by the usual scour baths. A still further object is to provide an improved method for the conditioning of yarns, particularly those composed of or containing organic derivatives of cellulose such as cellulose acetate, whereby the yarn is rendered soft and pliable and capable of employment in a variety of textile operations where complicated designs or stitches are employed. Still another object is to provide new chemical compounds having the structure and properties discussed below. Other objects will appear hereinafter.

These objects are accomplished by the following invention which, in its broader aspects, comprises the discovery that tetrahydrofurfuryl ethers having the general formula:



where R is an alkyl, alkoxyalkyl, hydroxyalkyl, hydroxyalkoxyalkyl, aralkyl, or aryl group which may be substituted with other groups such as tetrahydrofurfuryl, etc. may be used as yarn conditioning agents and particularly as softening agents with or without the addition of animal, mineral or vegetable oils in the treatment of yarns composed of or containing organic derivatives of cellulose. We have found that these compounds have a slight solvent and/or softening action on cellulose organic derivatives yarns which renders such yarns soft and pliable without at the same time having too drastic a solvent action thereon. As indicated above, included within the broad scope of our invention are the tetrahydrofurfuryl ethers having the general formula:



where R is monoalkoxyalkyl, polyalkoxyalkyl, or the tetrahydrofurfuryl nucleus.

In accordance with the invention these compounds may be applied directly to the yarn during or after spinning, or may be added to the spinning solution itself. We have found that these compounds have exceptional solvent powers which enable them to dissolve mineral oils and blown and unblown, drying and semi-drying vegetable and animal oils and accordingly, and they may be, and preferably are, employed as

ingredients of yarn conditioning or lubricating formulas in conjunction with agents which function wholly or partially as lubricants.

In the following examples and description, we have set forth several of the preferred embodiments of our invention, but they are included merely for purposes of illustration and not as a limitation thereof.

The ethers of tetrahydrofurfuryl alcohol of the type indicated above are prepared as described by Kirner, J. American Chemical Society 52, 3251 (1930). With respect to the preparation of the alkoxy alkyl compounds such as tetrahydrofurfuryl ethoxyethyl ether and tetrahydrofurfuryl methoxymethyl ether, the general method of Ashburn, Collett, and Lazell, J. American Chemical Society, 57, 1862 (1935) may be modified and used for this purpose. The preparation of typical compounds of this class in accordance with such technique may be carried out as follows:

*Preparation of tetrahydrofurfuryl ethoxyethyl ether*

25 1 mole of sodium is dissolved in 4 moles tetrahydrofurfuryl alcohol and the solution treated in the cold with 1 mole  $\beta$ -bromoethyl ether. The mixture is stirred 2 hr. at room temperature and 1 hr. on the steam bath to complete the reaction. The precipitated salt is filtered out and the filtrate worked up to give 55 gm. of ether, B. P. 100-110°/17 mm.

*Preparation of tetrahydrofurfuryl methoxymethyl ether*

35 In similar fashion to above, 1 mole of sodium is dissolved in 4 moles tetrahydrofurfuryl alcohol and treated with 1 mole of chloromethyl ether, stirring at 50° for 3 hr. The desired product is obtained as a liquid, B. P. 130-140°/20 mm.

*Preparation of  $\beta,\beta'$ -tetrahydrofurfuryl ethyl ether*

23 gm. (1.0 g. at) sodium are dissolved in 250 cc. tetrahydrofurfuryl alcohol. Then 72 gm. of  $\beta,\beta'$ -dichloroethyl ether are added with stirring 45 at a temperature above 50° C. The reaction mixture is heated for 4 hr. at 100° or above. Catalysts such as copper oxide, acetate, copper, etc., may be used. The salt is filtered out and the reaction product distilled. Distillation yields 70-130 gm. of  $\beta,\beta'$ -tetrahydrofurfuryl ethyl ether boiling at 213-215°/18 mm.

The above reaction may be run in presence of halogen acid removing compound. In addition to this there is obtained a good yield of a compound 55 having the formula:



60 boiling at 102-4°/8 mm.

Our invention will be more readily understood by reference to the following examples in which the use of tetrahydrofurfuryl ethers as yarn softening agents is described.

*Example I.*—Yarn designed for knitting and composed of cellulose acetate is treated by applying thereto tetrahydrofurfurylmethyl ether by means of an applicator roll, application being 70 conveniently carried out as the yarn emerges from the spinning cabinet or as it passes from bobbin to bobbin. The amount of the composition applied may run from 4-25% by weight of the yarn.

75 If the yarn is intended for weaving, the same

general procedure may be followed, except that the amount of the conditioning agent added to the yarn is only about 1-5%.

*Example II.*—A conditioning liquid having the following composition:

|                          | Percent |
|--------------------------|---------|
| Tetrahydrofurfuryl ether | 70      |
| Olive oil                | 30      |

10 applied to cellulose acetate yarn intended for knitting purposes. The amount of the conditioning liquid in this case is from 1-15% and the filaments or fibers thus treated are found to be quite soft and pliable and give improved results in knitting operations.

15 Other examples of yarn conditioning composition which may be applied to various types of yarn, particularly those composed of or containing cellulose organic derivatives such as cellulose acetate, cellulose acetate propionate and others in accordance with our invention and which render such yarn soft and pliable and well-adapted for 20 various textile operations particularly knitting, are the following:

|                                 | Percent |
|---------------------------------|---------|
| Tetrahydrofurfuryl propyl ether | 60      |
| Blown olive oil                 | 40      |

|                                | Percent |
|--------------------------------|---------|
| Tetrahydrofurfuryl butyl ether | 70      |
| Light mineral oil              | 30      |

|                               | Percent |
|-------------------------------|---------|
| Tetrahydrofurfuryl amyl ether | 30      |
| Neat's-foot oil               | 70      |

|                                 | Percent |
|---------------------------------|---------|
| Tetrahydrofurfuryl benzyl ether | 20      |
| Blown neat's-foot oil           | 30      |
| Sulfonated olive oil            | 20      |
| White mineral oil               | 10      |
| Oleic acid                      | 10      |
| Ethanolamine                    | 3       |
| Water                           | 45      |

|                                | Percent |
|--------------------------------|---------|
| Tetrahydrofurfurylmethyl ether | 20      |
| Sperm oil                      | 50      |
| Laurol                         | 60      |
|                                | 20      |

|                                | Percent |
|--------------------------------|---------|
| Tetrahydrofurfuryl ethyl ether | 20      |
| Blown sperm oil                | 30      |
| Sulfonated castor oil          | 20      |

|                                 | Percent |
|---------------------------------|---------|
| Tetrahydrofurfuryl methyl ether | 10      |
| Sulfonated olive oil            | 5       |
| Gelatin                         | 5       |
| Water                           | 80      |
|                                 | 75      |

60 *Example IX.*—A 20% solution of cellulose acetate in acetone in which is incorporated 1-25% by weight of tetrahydrofurfuryl cetyl ether of the cellulose acetate is extruded through fine orifices into an evaporative atmosphere. The filaments thus produced are pliable and suitable for knitting.

65 Other examples of yarn conditioning agents which may be applied to yarn in accordance with our invention are the following:

|                                 | Percent |
|---------------------------------|---------|
| Tetrahydrofurfuryl methyl ether | 10      |
| Sulfonated olive oil            | 5       |
| Gelatin                         | 5       |
| Water                           | 80      |
|                                 | 75      |

## Example XI

## Percent

|                                   |    |
|-----------------------------------|----|
| Water                             | 80 |
| Water soluble cellulose ester     | 5  |
| 5 Tetrahydrofurfuryl methyl ether | 10 |
| Diethylene glycol                 | 5  |

As indicated above, the alkoxy ethers derivable from tetrahydrofurfuryl alcohol are also particularly valuable as softening and conditioning agents for yarns composed of or containing organic derivatives of cellulose such as cellulose acetate, cellulose acetate propionate, etc. The following examples will further illustrate the use of these compounds:

15 *Example XII.*—A mixture of 40 parts of tetrahydrofurfuryl- $\beta$ -ethoxyethyl ether and 60 parts of blown olive oil is applied to cellulose acetate yarn by means of a bath, wick, roll, or spray application. If the yarn is intended for knitting, the amount of the applied compound may run from 4-25% by weight of the yarn. If the yarn is intended for weaving, the amount may vary between 1% and 5% by weight of the yarn.

20 Cellulose acetate filaments or fibers treated in this manner are found to be quite soft and pliable and give improved results in various textile operations such as weaving, knitting, etc.

Other examples of suitable conditioning liquids in accordance with our invention are the following:

30 *Example XIII.*—A conditioning liquid is made up as follows:

## Percent

|                                    |    |
|------------------------------------|----|
| Tetrahydrofurfuryl oxymethyl ether | 70 |
| Olive oil                          | 30 |

and applied to textile materials such as silk, wool, cellulose acetate, viscose, etc. as described in Example I. If the yarn is intended primarily for knitting, the amount of conditioning liquid applied may vary from 4-25% by weight of the yarn, and if the yarn is intended for weaving, the amount of liquid applied may vary from 1-5% by weight of the yarn.

45 *Example XIV.*—A conditioning liquid is made up as follows:

## Percent

|                                                  |    |
|--------------------------------------------------|----|
| $\beta$ -Tetrahydrofurfuryl oxyethyl vinyl ether | 60 |
| Blown olive oil                                  | 40 |

## Example XV

## Percent

|                                                       |    |
|-------------------------------------------------------|----|
| $\beta$ , $\beta$ '-Ditetrahydrofuryloxydiethyl ether | 70 |
| Light mineral oil                                     | 30 |

## Example XVI

## Percent

|                                                                 |    |
|-----------------------------------------------------------------|----|
| $\beta$ '-Ethoxy- $\beta$ -ethoxyethyl tetrahydrofurfuryl ether | 30 |
| Neat's-foot oil                                                 | 70 |

## Example XVII

## Percent

|                                              |    |
|----------------------------------------------|----|
| Tetrahydrofurfuryl- $\alpha$ -glyceryl ether | 20 |
| Sperm oil                                    | 60 |
| Lauroil                                      | 20 |

## Example XVIII

## Percent

|                                      |    |
|--------------------------------------|----|
| Tetrahydrofurfuryl ethoxyethyl ether | 50 |
| Blown sperm oil                      | 30 |
| Sulfonated castor oil                | 20 |

70 *Example XIX.*—A 20% solution of cellulose acetate in acetone in which is incorporated 1-25% by weight of the cellulose acetate of tetrahydrofurfurylmethoxymethyl ether is extruded through fine orifices into an evaporative atmos-

sphere. The filaments thus produced are wound or twisted and wound. Yarns produced from filaments thus prepared are pliable and suitable for knitting.

Still further examples of yarn conditioning agents which may be applied to yarn are the following:

Example XX.—A conditioning liquid is made up as follows:

|                                                |    |
|------------------------------------------------|----|
| Water                                          | 80 |
| Gelatin                                        | 5  |
| Tetrahydrofurfuryl- $\beta$ -ethoxyethyl ether | 10 |
| Sulfonated olive oil                           | 5  |

## Example XXI

## Percent

|                                                                    |    |
|--------------------------------------------------------------------|----|
| Water                                                              | 80 |
| Water soluble cell. ester                                          | 5  |
| Tetrahydrofurfuryl- $\beta$ '-ethoxy- $\beta$ '-ethoxy ethyl ether | 10 |
| Diethylene glycol                                                  | 5  |

As will be apparent from the above examples and description, the conditioning agents of our invention may be applied by a wide variety of methods. For example, we may employ the agent as an ingredient of the spinning dope from which the filaments are formed, the amount of the agent so employed depending upon a number of factors, such as the particular cellulose derivative used in making the yarn, the solvent or solvent combination used in making up the spinning solution, and the degree of softness or pliability desired in the yarn, etc.

If the conditioning agent is to be applied to the yarn after spinning, this may be done by bringing the yarn in contact with a wick, roll, or felt wet therewith or the liquid may be applied by immersion, spray, or otherwise. The particular point at which the liquid is applied may vary. It may, for example, be applied to the yarn inside or outside the spinning cabinet, between the guide and godet roll, between the godet or other roll or guide and the point of winding and/or twisting. In some cases, the liquid may even be applied to the yarn after winding onto cones, spools, bobbins, or the like or by the so-called "bobbin to bobbin" method. In the case of staple fiber manufacture, the liquid may be applied to the yarn prior to, or after cutting into staple lengths.

The amount of the agent so employed will vary widely depending upon the results desired, the specific nature of the material to which the agent is applied, the use to which the yarn is eventually to be put and other factors. For example, in a given case where a cellulose organic acid ester yarn, such as a yarn composed of cellulose acetate, is intended for knitting, about 4 to 25% or more by weight, based on the weight of the dry yarn, may be satisfactory, while if the yarn is intended for weaving, the amount may vary between about 1 and 5%.

Although in the above examples we have referred primarily to yarn treating compositions containing only the conditioning agent and an oil, other ingredients such as solvents, non-solvents, emulsifying agents, blending agents and the like, may be added within the scope of our invention. Likewise, various dyes or other coloring matter may be included in case it is desired to permanently or fugitively tint or dye the material undergoing treatment.

Although we have found it convenient to illustrate our invention by reference to composi-

tions containing specific percentages of the various ingredients, these percentages may vary widely depending upon the particular purpose for which the composition is intended. For example, if it is desired to control the solvent or softening action of the conditioning agent, the amount of the agent may be adjusted as, for example, by reducing the amount of the agent and correspondingly increasing the amount of oil or 10 other ingredient.

While we have described our invention with particular reference to the treatment of yarns composed of organic derivatives of cellulose such as cellulose acetate, the conditioning agents and 15 formulae described herein are applicable to the conditioning of many other types of cellulose derivative yarns such as those composed of or containing cellulose propionate, cellulose butyrate, cellulose acetate propionate, cellulose acetate 20 butyrate, ethyl cellulose, methyl cellulose, benzyl cellulose and others, as well as to the conditioning of silk, wool, cotton, viscose and other natural or artificial materials.

The term "yarn" as used herein and in the 25 claims is to be understood as including a single filament, a plurality of filaments associated into the form of a thread, either of high or low twist, single or multiple threads associated or twisted together, composite threads composed of a mixture of natural and artificial filaments or a composite thread formed by twisting together individual strands of natural or artificial materials, as well as cut staple fibers produced from natural and/or artificial filaments or threads and 30 spun yarn produced from such staple fibers.

As indicated above, the yarn conditioning agents of our invention are exceptionally good solvents for a wide variety of mineral, blown and unblown, drying and semi-drying animal and 40 vegetable oils such as cottonseed, olive, castor, neat's-foot, sperm and other oils. This enables them to be used with any of such oils in making up a variety of yarn treating formulae of varying composition.

45 The yarn conditioning method and compositions of our invention possess many outstanding advantages. The fundamental and outstanding characteristic of the agents employed in accordance with the invention is their ability to soften 50 yarns, especially those composed of or containing organic derivatives of cellulose such as cellulose acetate and render them soft and pliable and amenable to various textile operations, especially operations such as those involved in weaving 55 and knitting where complicated designs or stitches are employed, without too drastic an action on the yarn material.

Another outstanding characteristic of these 60 compounds is their exceptional solvent power for a wide variety of mineral, animal and vegetable oils and their ability to act as lubricating assistants in conjunction with these oils when applied to such yarns. In addition, due to their solubility in water, they may be readily removed 65 from yarns and fabrics by means of the usual aqueous scour baths. By employing the yarn conditioning agents and method of our invention as herein described, one is enabled to obtain highly satisfactory results in the manufacture 70 of yarns and woven fabrics and especially the production from these yarns of closely knit fabrics free from defects such as pin holes, stitch distortion, laddering and the like.

What we claim and desire to secure by Letters 75 Patent of the United States is:

1. The process of conditioning yarn to render it more amenable to textile operations including knitting, weaving, spinning and the like which comprises applying thereto a lubricating and softening composition containing a tetrahydrofurfuryl ether having the general formula: 5



10

where R is an alkyl, alkoxyalkyl, hydroxyalkyl, hydroxyalkoxyalkyl, aralkyl, or aryl group.

2. The process of conditioning yarn composed of or containing organic derivatives of cellulose to render it more amenable to textile operations including knitting, weaving, spinning and the like which comprises applying thereto a lubricating and softening composition containing a tetrahydrofurfuryl ether having the general formula: 15



20

where R is a monoalkoxyalkyl, polyalkoxyalkyl or the tetrahydrofurfuryl nucleus. 25

3. The process of conditioning yarn composed of or containing cellulose acetate to render it more amenable to textile operations including knitting, weaving, spinning and the like, which comprises applying thereto a lubricating and softening composition containing a tetrahydrofurfuryl ether having the general formula: 30



35

where R is an alkyl, alkoxyalkyl, hydroxyalkyl, hydroxyalkoxyalkyl, aralkyl, or aryl group.

4. The process of conditioning yarn composed of or containing cellulose acetate to render it more amenable to textile operations including knitting, weaving, spinning, and the like, which comprises applying thereto a lubricating and softening composition containing a tetrahydrofurfuryl ether having the general formula: 40



45

where R is monoalkoxyalkyl, polyalkoxyalkyl, or the tetrahydrofurfuryl nucleus. 50

5. The process of conditioning yarn composed of or containing cellulose acetate to render it more amenable to textile operations including knitting, weaving, spinning and the like, which comprises applying thereto a lubricating and softening composition containing a tetrahydrofurfuryl ether having the general formula: 55



60

where R is an alkyl, alkoxyalkyl, hydroxyalkyl, hydroxyalkoxyalkyl, aralkyl, or aryl group and a textile lubricant. 65

6. The process of conditioning yarn composed of or containing cellulose acetate to render it more amenable to textile operations including knitting, weaving, spinning and the like, which comprises applying thereto a lubricating and softening composition containing tetrahydrofurfuryl ethyl ether. 70

7. The process of conditioning yarn composed of or containing cellulose acetate to render it 75

more amenable to textile operations including knitting, weaving, spinning and the like, which comprises applying thereto a lubricating and softening composition containing tetrahydrofurfuryl benzyl ether.

8. A conditioning agent for rendering yarns more amenable to textile operations including knitting, weaving, spinning, and the like which comprises a tetrahydrofurfuryl ether having the general formula:



15 where R is an alkyl, alkoxyalkyl, hydroxyalkyl, hydroxyalkoxyalkyl, aralkyl, or aryl group.

9. A conditioning agent for rendering yarns more amenable to textile operations including knitting, weaving, spinning, and the like which comprises a tetrahydrofurfuryl ether having the general formula:



25 where R is monoalkoxyalkyl, polyalkoxyalkyl, or the tetrahydrofurfuryl nucleus.

10. A conditioning agent for rendering textile yarns composed of or containing organic derivatives of cellulose more amenable to textile operations including knitting, weaving, spinning, and the like which comprises a tetrahydrofurfuryl ether having the general formula:



35 where R is an alkyl, alkoxyalkyl, hydroxyalkyl, hydroxyalkoxyalkyl, aralkyl, or aryl group and a textile lubricating oil.

11. A conditioning agent for rendering textile yarns composed of or containing organic derivatives of cellulose more amenable to textile operations including knitting, weaving, spinning, and the like which comprises a tetrahydrofurfuryl ether having the general formula:



50 where R is monoalkoxyalkyl, polyalkoxyalkyl, or the tetrahydrofurfuryl nucleus.

12. A conditioning agent for rendering yarns composed of or containing cellulose acetate more amenable to textile operations including knitting, weaving, spinning, and the like, containing tetrahydrofurfuryl ethyl ether.

60 13. A conditioning agent for rendering yarns composed of or containing cellulose acetate more amenable to textile operations including knitting, weaving, spinning, and the like containing tetrahydrofurfuryl benzyl ether.

14. Textile yarn amenable to textile operations including knitting, weaving, spinning and the like impregnated with a lubricant containing a tetrahydrofurfuryl ether having the general formula:



where R is an alkyl, alkoxyalkyl, hydroxyalkyl, hydroxyalkoxyalkyl, aralkyl, or aryl group.

15. Textile yarn amenable to textile operations including knitting, weaving, spinning, and the like impregnated with a lubricant containing a tetrahydrofurfuryl ether having the general formula:



20 where R is monoalkoxyalkyl, polyalkoxyalkyl, or the tetrahydrofurfuryl nucleus.

16. Textile yarns composed of or containing cellulose acetate amenable to textile operations including knitting, weaving, spinning, and the like, impregnated with a lubricant comprising tetrahydrofurfuryl ethyl ether.

17. Textile yarns composed of or containing cellulose acetate amenable to textile operations including knitting, weaving, spinning and the like, impregnated with a lubricant comprising tetrahydrofurfuryl benzyl ether.

18. As new chemical compounds, tetrahydrofurfuryl ethers having the formula:



40 where R is monoalkoxyalkyl, polyalkoxyalkyl, or the tetrahydrofurfuryl nucleus.

19. As new chemical compounds, alkoxyalkyl ethers of tetrahydrofurfuryl alcohol selected from the group consisting of tetrahydrofurfuryl methoxymethyl ether and tetrahydrofurfuryl- $\beta$ -hydroxyethyl ether.

45 20. The process of conditioning yarn composed of or containing cellulose acetate to render it more amenable to textile operations including knitting, weaving, spinning and the like, which comprises applying thereto a lubricating and softening composition containing  $\beta,\beta'$ -ditetrahydrofuryloxydiethyl ether.

21. A conditioning agent for rendering yarns composed of or containing cellulose acetate more amenable to textile operations including knitting, weaving, spinning and the like containing  $\beta,\beta'$ -ditetrahydrofuryloxydiethyl ether.

55 22. Textile yarns composed of or containing cellulose acetate amenable to textile operations including knitting, weaving, spinning, and the like, impregnated with a lubricant comprising  $\beta,\beta'$ -ditetrahydrofuryloxydiethyl ether.

JAMES G. McNALLY.  
JOSEPH B. DICKEY.